

# United States Patent [19]

Efird

[11] 3,766,025

[45] Oct. 16, 1973

[54] REPAIRING ELECTROLYTIC CELLS

3,428,545 2/1969 Johnson ..... 204/243 R X  
3,457,149 7/1969 Johnson ..... 204/243 R X  
3,514,520 5/1970 Bacchiega et al. .... 204/243 R X

[75] Inventor: **Gaston C. Efird, Albermarle, N.C.**

[73] Assignee: **Aluminum Company of America, Pittsburgh, Pa.**

[22] Filed: **June 30, 1972**

[21] Appl. No.: **268,180**

[52] U.S. Cl. .... 204/67

[51] Int. Cl. .... C22d 3/12

[58] Field of Search..... 204/67

## [56] References Cited

### UNITED STATES PATENTS

2,971,899 2/1961 Hannink et al. .... 204/243 R X

*Primary Examiner*—John H. Mack

*Assistant Examiner*—D. R. Valentine

*Attorney*—Edward B. Foote

[57]

## ABSTRACT

Holes which develop in the base of an electrolysis chamber in an electrolytic cell and expose a metal member in the said base to contact by liquid material in the chamber are repaired during operation of the cell by feeding into the liquid a granular material which settles through the liquid and plugs the hole.

4 Claims, No Drawings

## REPAIRING ELECTROLYTIC CELLS

This invention relates to repairing the electrolysis chamber of an electrolytic cell, and relates particularly to procedures for effecting such repair during operation of the cell.

## BACKGROUND OF THE INVENTION

Aluminum is conventionally produced commercially by the well-known Hall-Heroult process, in which electrolysis of alumina dissolved in molten fluorides — principally cryolite — is carried out in electrolysis chambers having an electrically conductive lining surrounded by insulation and a metal sheath, there being one or more anodes disposed above the cell and extending into the alumina-fluoride electrolytic bath. A layer of molten aluminum in the cell rests on the lower portion of the electrolysis chamber and acts as the cell cathode. The above-mentioned lining ordinarily consists of baked carbon, either in monolithic form or in blocks bonded together with a carbonaceous binder. Metal (e.g., iron, steel or copper) collector bars embedded in the carbon lining and connected externally to the cathode bus conduct electric current from the cell. U. S. Pat. Nos. 2,528,905, 2,593,751, 2,874,103, 2,874,110, 3,236,753, 3,494,851 and 3,514,520 disclose cells of the type referred to above.

The invention will be described below in connection with electrolytic cells for use in the Hall-Heroult process for the production of aluminum, although it is also applicable to cells for other electrolytic processes, for example, the well-known "three-layer" process for electrolytic purification of aluminum. U. S. Pat. Nos. 1,534,316, 1,534,317 and 2,582,661 disclose the three-layer process and cells of the type used in operation of it.

As is pointed out in "Formation of Potholes in Bottom Linings of Hall Cells," by Dell, Peterson and rumble, *Journal of Metals*, September 1968, pages 55-58, a common problem encountered in the operation of electrolytic cells for the production of aluminum is the gradual formation of "portholes" in the lower portion of the electrolysis chamber. Such holes are eroded areas, shaped roughly like inverted cones, which develop downward from the molten pool of aluminum resting on the electrolysis chamber base, and gradually become deep enough to penetrate to a metal collector bar embedded in that base, permitting molten aluminum to contact the bar and dissolve metal therefrom, with resultant contamination of the aluminum, as well as impairment of the current efficiency of the cell. The collector bar area thus contacted by the molten aluminum is referred to herein as the exposed area of the bar.

Penetration of a pothole to a metal collector bar embedded in the base of the electrolysis chamber can be detected by periodic analysis of the molten aluminum in the cell to determine whether it has been contaminated by collector bar metal. When such contamination is observed, it has been the practice to discontinue operation of the cell, drain the electrolytic bath and molten aluminum from it, and replace or repair the electrolysis chamber, all at substantial expense and interference with production of metal in the cell.

## The Invention

It is the object of this invention to provide a convenient and economical method of repairing holes in the base of an electrolysis chamber of an electrolytic cell during continued operation of the cell.

In accordance with the invention, upon finding that a hole in the base of the electrolysis chamber of an electrolytic cell has penetrated to a metal bar embedded in that base, the location of the hole is ascertained. This may be done by probing the bottom of the electrolysis chamber with a metal rod inserted downward through the electrolytic bath layer and the molten aluminum layer beneath it. Locating the hole in that manner can be facilitated by first identifying the particular bar affected, which can be accomplished by measuring the current loading of the respective collector bars in the lining with a suitable ammeter. A current loading outside normal range on a particular collector bar is an indication that it is the bar with which molten aluminum in the chamber is in contact. The location of the hole can then be determined by probing the bottom of the electrolysis chamber in the area adjacent the affected collector bar.

When the hole in the lining has been thus located, granular material having sufficient density for it to settle through the electrolytic bath and the molten aluminum layer beneath it is fed into the bath in the area over the hole, whereupon the granular material settles into the hole. Sufficient granular material is fed into the hole in this manner to cover the exposed area of the collector bar thoroughly and prevent further access of molten aluminum thereto, thereby forestalling further attack on the metal bar by the aluminum. Following introduction of the desired amount of granular material into the hole, it is desirable to pack it securely in place by tamping it with a metal rod. Shielding of the granular material by the liquid metal layer prevents or minimizes its dissolution in the molten electrolytic bath.

The granular material employed may be in the form of balls, chips, pellets, or the like of a material which is not readily soluble in, or melted by, the electrolytic bath or the molten aluminum. Pellets of alumina are particularly suitable for the purpose, since they do not introduce undesirable impurities into the bath or the aluminum, and are capable of withstanding prolonged contact with the molten aluminum. Pellets of alpha alumina are preferred, since alpha alumina is less readily soluble in the electrolytic bath than other crystalline or amorphous forms of alumina. However, granules of such other refractory materials such as silicon carbide and boron nitride, can also be used in carrying out the invention.

The above-mentioned steps of locating the hole in the base of the electrolysis chamber, feeding granular material through the molten bath and molten aluminum layers to fill the hole with such material, and tamping that material, can all be carried out without discontinuing the electrolytic production of aluminum in the cell. Moreover, use of the procedures described above make it possible to extend the life of the electrolysis chamber, and also affords increased latitude in scheduling replacement of electrolysis chambers of cells in plants using a large number of such cells, as is normally the situation in modern plants for the production of aluminum.

As an example of the invention, in producing aluminum in an electrolytic cell with an electrolysis chamber having a carbon bottom and side walls, horizontally disposed iron collector bars embedded in the chamber bottom, and a number of pre-baked carbon electrodes suspended in a bath of molten fluorides and dissolved alumina, upon detecting an increase in the iron content of aluminum produced in the cell to about 0.8 percent by weight from a normal level of about 0.2 percent, the current loading of the various iron collector bars was checked with an ammeter and it was found that the loading of one of the bars was unusually high. Cell anodes over that collector bar were removed temporarily from the electrolytic bath, without discontinuing feeding electric current to the cell through remaining anodes of the cell, and upon probing the electrolysis chamber floor in the area adjacent that bar with a steel rod inserted through the molten layers of electrolytic bath and aluminum, a pothole extending to the collector bar was located in the chamber floor.

Small balls (approximately three-fourths inch in diameter) of alpha alumina, with a specific gravity of about 4, and mixed with fine particles of such alpha alumina, were poured into the electrolytic bath in the area above the pothole. The mixture settled into the pothole, displacing the molten aluminum therein and covering the exposed area of the collector bar. The mixture in the hole was next tamped into place with a steel rod, after which the above-mentioned removed anodes were put back into place and were again used

to supply current to the cell. After two weeks of continued operation of the cell in a normal manner, the molten aluminum in the cell was analyzed to determine its iron content, which content was found to be about 0.1 percent. The current loading of the above-mentioned collector bar at that time was at normal range.

I claim:

- 10 1. In the operation of an electrolytic cell having an electrolysis chamber with a bottom on which liquid is supported, the said bottom having current-conducting metal members embedded therein beneath the said liquid, the method of repairing a hole in the said chamber bottom which exposes an area of one of said members to contact by said liquid, which comprises the steps of determining the location of the said hole, and feeding into the liquid in the area over the hole sufficient granular material which settles into the said hole to cover the said exposed area and prevent access thereto by said liquid.
- 20 2. The method of claim 1 in which the location of the said hole is determined by probing the said bottom in the area adjacent a current-conducting member exhibiting a higher current loading than normal therefor.
- 25 3. The method in accordance with claim 1, in which the cell is one for the electrolytic reduction of alumina to aluminum in a fused fluoride bath, and the said liquid consists of molten aluminum.
4. The method in accordance with claim 1, in which the said granular material consists of alumina.

\* \* \* \* \*

30

35

40

45

50

55

60

65